

## UNITED STATES PATENT OFFICE

RICHARD GEORGE WOODBRIDGE, OF WILMINGTON, DELAWARE, ASSIGNOR TO E. I. DU PONT DE NEMOURS & COMPANY, OF WILMINGTON, DELAWARE, A CORPORATION OF DELAWARE

## PROPELLENT POWDER

No Drawing.

Application filed April 22, 1929. Serial No. 357,335.

This invention relates to a process of suppressing muzzle flash in guns and to an improved propellant powder having incorporated therein an amount of flash suppressing salt insufficient of itself to suppress muzzle flash, but which in combination with an added increment of flash suppressing salt will suppress muzzle flash to the extent desired without affecting the ballistics of the powder.

This application is a continuation in part of my copending applications Serial Nos. 81,086 and 269,881, filed January 13, 1926, and April 13, 1928, respectively.

The practice of adding packets of potassium chloride to the powder charge, principally at night, for the prevention of muzzle flash was known during the World War. It is also well known that relatively large additions of potassium chloride or other salts are required when the salt is added in this manner, and that these large additions of such salts seriously disturb the ballistics of the powder charge. There is the further disadvantage that the flashless results are accompanied by large volumes of white smoke. This is especially true because the amount of potassium chloride or like salt required to suppress muzzle flash when added in packet form may amount to 8 or 10%, and even more, of the weight of the powder charge.

In my co-pending application Serial No. 269,881, filed April 13, 1928, I have shown that flashless results may readily be obtained in a large number of guns with a propellant powder of the preferred composition

85 parts nitrocellulose of about 13.15% nitrogen  
10 parts dinitrotoluol  
5 parts dibutylphthalate  
1 part diphenylamine

45

in which there has been incorporated during the process of colloiding and mixing, as little as one part of potassium sulphate.

The flashless results obtained with the above powder are naturally accompanied by a certain amount of white smoke due in part to the potassium sulphate contained in the powder and also to the saltpetre contained in the black powder used in the primer or ignition pad, or both. This amount of smoke is not large or objectionable in the smaller guns, as for example the 3" anti-aircraft, where the weight of powder charge is about five pounds and the primer contains only about 110 grains of black powder.

Powder of the above type is admirably suited for use in fixed ammunition as flashless results are obtained with relatively little smoke. However, as pointed out in my said co-pending application Serial No. 269,881, when flashless results are obtained in the 155 m/m G. P. F. gun with powder of the above mentioned type, a larger quantity of white smoke is produced. Of this quantity the smaller portion is due to approximately four (4) ounces of potassium sulphate present in the 25 pounds required weight of charge of powder containing 1% of potassium sulphate and the larger portion due to the six ounces of saltpetre contained in the eight ounces of black ignition powder used as an ignition charge to supplement the 21 grain primer.

The ever increasing use of aeroplanes and photography in modern warfare makes it

55

55

60

65

65

70

75

75

80

desirable to reduce the amount of smoke to a minimum. Muzzle flash in the daytime is not seriously objectionable, but visible or photographicable smoke in the daytime is 5 as highly objectionable as muzzle flash is at night.

An object of my invention is a process of eliminating muzzle flash.

Another object of my invention is an 10 proved powder which while exhibiting muzzle flash in the daytime may be readily made to give flashless results at night without at the same time seriously interfering with the ballistics of the powder charge, and further- 15 more without yielding excessive smoke which is so objectionable to gunners at any time.

A still further object of my invention is a nitrocellulose propellant powder which, besides being of greatly reduced hygroscopic- 20 ity, can be dried not only in air but also in hot water in order to more effectively and expeditiously remove the volatile solvents added for the purpose of assisting in the col- loiding of the nitrocellulose.

25 A still further object of my invention is to retain the advantages of my improved propellant powder as described in my co-pending applications Serial Nos. 81,086 and 269,881, aforesaid, only modifying its com- 30 position to the slightest degree in order to produce a powder which in certain guns will not give flashless results without the use of an additional quantity of a flash suppressing salt over and above that incorporated in the 35 powder in an insufficient amount to give flash- lessness.

These objects are accomplished by the following invention, in which I have discovered that a relatively small amount of a flash suppressing salt uniformly incorporated in the colloid is of great value in suppressing muzzle flash, as hereinafter described. By incorporating in the powder an insufficient quantity of a flash suppressing salt the powder 45 will invariably, preferably always, give rise to some muzzle flash. In this manner the objection to smoke during day time firings is overcome as the smoke is volatilized by the 50 flash.

However, the incorporation of some flash suppressing salt, although insufficient to suppress muzzle flash, will insure the uniform distribution of this small amount of the salt 55 throughout the powder gases. I have found, furthermore, that the addition to the powder charge of a relatively small additional amount of the salt will completely suppress muzzle flash. In this way flashless results 60 can readily be obtained at will either in day or night firings by the simple expediency of adding to the powder charge a small additional amount of the salt to that already incorporated in the colloid. In this way flash- 65 less results are obtained with practically no

change in velocity and pressure of the powder and at the same time with a minimum amount of smoke.

I have found that potassium salts answer this purpose very satisfactorily, although other flash suppressing salts, particularly the alkali metal salts, may be used as hereinafter more fully described. It will be apparent to those skilled in the art of ordnance that powder of the foregoing type is particularly suited to guns in which the powder is loaded separately in silk bags, because in this way an increment of potassium sulphate or other flash suppressing salt can be added to the 70 charge whenever flashless results are desired. 75

According to my invention disclosed in co-pending application Serial No. 269,881, if one part of potassium sulphate is incorporated in the powder flashless results on all 80 rounds would be obtained. This relatively small amount of potassium sulphate required to suppress muzzle flash when the salt is incorporated in the smokeless powder colloid is due to the uniform distribution of the 85 potassium sulphate throughout the powder and consequently throughout the volume of combustible powder.

I have now found that flashless results may be readily obtained with even smaller quantities of potassium sulphate, one-third to one-half parts, provided there be subsequently added to the powder charge an additional amount of potassium sulphate in the manner 90 95 subsequently described herein.

I have found that very desirable results may be obtained by incorporating in the powder approximately one-half of 1% (.5%) of an alkali salt that is non-hygroscopic up to 105 about 90% relative humidity at atmospheric temperature and that this amount of the salt has no harmful action on the ballistics of the powder.

The following illustrative example will 110 show one embodiment, but this is not to be taken in any way as a limitation of my invention: Powder of the following composition

115  
85 parts nitrocellulose of about 13.15% ni-  
trogen content  
10 parts dinitrotoluene  
5 parts dibutylphthalate  
1 part diphenylamine  
1/3 to 1/2 part of potassium sulphate

120  
125  
will invariably give rise to large luminous muzzle flash when fired in the 155 m/m G. P. F. gun with the 95 pound projectile, using the 21 grain primer with an eight ounce ignition pad of black sporting powder.

In order that my invention may be more clearly understood, reference is made to the 130

table of ballistic results and other data given below:

Table of ballistic results in the 155 m/m G. P. F. gun with 95 pound projectile. Primer used, 21 grains with an 8 ounce pad of black sporting powder as base igniter charge

|    | Composition of powder                                                                                                                    | Added increment of potassium sulphate                                                | Number of rds. | Weight of charge | Muzzle velocity ft./sec., mean | Mean pressure, lbs./sq. in. | Muzzle flash      | 70 |
|----|------------------------------------------------------------------------------------------------------------------------------------------|--------------------------------------------------------------------------------------|----------------|------------------|--------------------------------|-----------------------------|-------------------|----|
| 10 | 85 pts. N/C of 13.15% nitrogen<br>10 pts. dinitrotoluene<br>5 pts. dibutylphthalate<br>1 pt. diphenylamine<br>1/2 pt. potassium sulphate | None                                                                                 | 3              | 25 lbs. 14 ozs.  | 2344                           | 27,483                      | Large             | 75 |
|    | Same                                                                                                                                     | 2 ounces of 5 grain tablets of potassium sulphate contained in silk bag              | 3              | 26 lbs.          | 2363                           | 28,483                      | 1 large<br>2 none |    |
| 15 | Same                                                                                                                                     | 3 ounces of 5 grain tablets                                                          | 5              | 26 lbs.          | 2356                           | 28,130                      | None              | 80 |
|    | Same                                                                                                                                     | 4 ounces of nitrocellulose colloid containing 50% or 2 ounces of potassium sulphate  | 5              | 26 lbs.          | 2369                           | 29,040                      | None              |    |
| 20 | 85 pts. N/C of 13.15% nitrogen<br>10 pts. dinitrotoluene<br>5 pts. dibutylphthalate<br>1 pt. diphenylamine                               | 8 ounces of nitrocellulose, colloid containing 50% or 4 ounces of potassium sulphate | 5              | 26 lbs.          | 2392                           | 30,450                      | 3 large<br>2 none | 35 |

In the first four series of tests recorded in the foregoing table, the same kind of powder was used. The weight of charge selected for 25 the first firings gave results about 16 feet per second lower than the standard powder fired in comparison, which was made up in subsequent firings by the addition of two more ounces of powder.

30 In the second and third series of tests the potassium sulphate was added in the form of 5 grain compressed tablets, the total quantity being put into a silk bag and the bag tied on to the end of the bag loaded charge so 35 that it came next to the projectile. Two ounces of potassium sulphate added in this manner gave two flashless rounds out of three while three ounces of the salt gave five flashless rounds out of five.

40 In the fourth series of firings four ounces of an air dried nitrocellulose colloid containing 50% or two ounces of potassium sulphate were added in a silk bag and five flashless rounds obtained out of five. The smaller 45 amount of potassium sulphate required to suppress muzzle flash when added in the above manner I attribute to the fact that the potassium sulphate is gradually given up to the powder gases during the combustion of

50 the powder and is more uniformly distributed throughout the volume of gases. This method of obtaining more uniform distribution of the potassium sulphate throughout the powder gases comprises a particular feature of my invention.

The last series of firings in the table shows the combination of a powder not containing incorporated potassium sulphate with eight ounces of nitrocellulose colloid containing 50% or four ounces of incorporated potassium sulphate. Flashless results were obtained on only three rounds out of five whereas as shown in co-pending application 269,881 the same amount, four ounces or 1% of potassium sulphate, incorporated in the powder

ounces, of the nitrocellulose colloid containing 50% of potassium sulphate failed to give consistently flashless results, which I attribute to the fact that the potassium sulphate does not become uniformly distributed throughout the combustible gases.

As shown by the ballistic results obtained in the third and fourth series of firings shown in the above table, flashless results are obtained with practically no change in the ballistic results of the powder. Therefore, it is unnecessary to make any allowance for change in velocity of the projectile as such allowance would come well within the usual variation experienced in measuring velocities by the chronograph. Furthermore, it is unnecessary to add to or subtract from the amount of powder representing the standard weight of charge. It is only necessary to add to the powder charge the necessary increment of potassium sulphate which as a matter of convenience, may be contained in a silk bag, of special color if desired, and simply tied on to the end of the charge.

The manufacture of the powder requires no special skill over known methods, the following example being illustrative:

The nitrocellulose is dehydrated with denatured ethyl-alcohol of suitable grade and then colloided in a suitable mixer with the addition of ether. There is added in the ether or directly to the mixer, the dinitrotoluene and the dibutylphthalate. Due to the solvent action of the latter two ingredients, less alcohol and ether are required than is usually the case for nitrocellulose powders not containing these ingredients. The potassium sulphate is uniformly and finely ground in a ball mill or other type of mill to a fineness sufficient to pass through a wire screen of eighty meshes to the inch. However, I do not limit myself to this fineness. Diphenylamine is usually added as a stabilizer and is usually dissolved in the ether.

The colloid may be pressed either in tubular grains with one or more perforations or in the solid grain, or in the ribbon or strip form of grain. The grains of powder are given 5 thorough solvent recovery treatment before the final drying, which may be in air or hot water at a temperature not in excess of 60° C., although a higher temperature may be used without affecting the chemical stability 10 of the powder.

While I prefer to use a standard composition containing

85 parts nitrocellulose of about 13.15% nitrogen  
15 10 parts dinitrotoluol  
5 parts dibutylphthalate  
1 part diphenylamine  
1/3 to 1/2 part potassium sulphate

20 it should be understood that I do not limit myself to these proportions or to these ingredients. For example, the nitrocellulose I may use may be a mixture of the type soluble in ether-alcohol with the type insoluble in 25 ether-alcohol mixture (two parts ether to one part ethyl alcohol), and of a higher or lower nitrogen content than 13.15%, or it may be entirely of the soluble type, having a nitrogen content between about 12.0 and 30 12.80%.

The dinitrotoluene may be decreased or increased, or substituted by other nitro compounds.

The dibutylphthalate may also be increased or decreased or substituted by other cooling agents which are solvents for nitrocellulose such as those mentioned in my co-pending application No. 81,086 filed January 13, 1926.

40 The potassium sulphate incorporated in the propellant powder will be in the neighborhood of 1/3 to 1/2% for the 155 m/m G. P. E. gun; for other guns having different characteristics it may be greatly in excess 45 of this amount. It should be understood that it is the intention to incorporate in the powder as much potassium sulphate as possible, without obtaining flashless results, and that the best amount to use for each gun can 50 readily be determined by experimentation.

The potassium sulphate added to the powder charge is preferably in the form of tablets, which prevents dusting that would occur if powdered potassium sulphate were used. The 55 potassium sulphate may also be contained in a nitrocellulose, cellulose ester or other film. The silk of the powder bag may be weighted with the potassium sulphate. However, I prefer to incorporate the potassium sulphate 60 in a nitrocellulose colloid in order that as the colloid gradually burns, the potassium sulphate will be gradually given up to the powder gases and in this manner there will be secured a more uniform distribution of the potassium sulphate throughout the powder

gases. The colloid containing the potassium sulphate may be similar in composition to my preferred composition for the propellant powder, as for example

70 85 parts nitrocellulose of 13.15% nitrogen  
10 parts dinitrotoluene  
5 parts dibutylphthalate  
1 part diphenylamine  
50 parts potassium sulphate

75 The above colloid may be manufactured in exactly the same manner as the propellant powder itself, except that it should preferably be air dried. The colloid may be pressed in the form of strips, rolls or tubes with one or more perforations, and cut into convenient grains, which need not be of the same form or thickness as the propellant powder.

80 In describing the above composition of nitrocellulose colloid containing potassium sulphate, it should be understood that I do not limit myself to this composition or to composition of the nitrocellulose type, and may incorporate the potassium sulphate in 85 powders of nitroglycerine or other type.

85 While I prefer to use propellant powder of the nitrocellulose type, and particularly powder of the composition described in my co-pending applications Serial Nos. 81,086 and 269,881, it should be understood that I 90 do not limit my invention to powder of any particular composition. It will be apparent that I can incorporate in any kind of powder, whether of the nitrocellulose or nitroglycerine or some other type, potassium sulphate in an insufficient amount to suppress muzzle flash, and that I can add to the powder charge the additional increment of potassium sulphate required to suppress muzzle 95 flash.

100 In place of potassium sulphate, either in the propellant powder or the flashless increment, or both, I may use some other alkali metal salt such as potassium nitrate, potassium oxalate, potassium chloride, sodium chloride, sodium nitrate, sodium oxalate, etc., but I prefer to use those salts which are non-hygroscopic up to about 90% relative humidity at atmospheric temperature and also 105 which have no harmful action on the stability of the powder. It is obvious that in the case of the flashless increment if the salt is added loose or in tablet form it need not be a salt without any action on the stability of the nitrocellulose or powder, as the salt if contained in a silk bag, would not come in contact with the propellant powder.

110 This invention is applicable to obtaining flashless results in cannons, particularly the larger guns which do not use fixed ammunition, but in which the projectile and powder charge are loaded separately.

115 The invention overcomes the objection to the smoke produced by flashless powders, particularly in the large guns, by providing 120

125

first, a powder which is not flashless for use in day firings, but which powder contains an insufficient amount of flash suppressing salt and can be readily made flashless at night by the addition of a very small increment of the same or other flash suppressing salt.

It will therefore be seen from the foregoing that my invention possesses the following advantages among others:

- 10 Flashless results are obtained with practically no change in the ballistic results given by the powder, as the flash suppressing increment is so small as to have no effect on the ballistics of the powder.
- 15 Flashless results are obtained at will, either in day or night firings, by the simple expediency of adding to the powder charge a packet of the flash suppressing salt or colloid containing the salt.
- 20 These flashless results are obtained with a minimum amount of smoke.

As many apparently widely different embodiments of this invention may be made without departing from the spirit thereof, it is to be understood that I do not limit myself to the foregoing examples or descriptions except as indicated in the following patent claims.

I claim:

- 30 1. The process of suppressing muzzle flash which comprises incorporating in propellant powder a small quantity of an alkali metal salt insufficient in itself to eliminate muzzle flash, and subsequently adding to the charge an increment of a flash suppressing alkali metal salt in quantity sufficient in combination with the alkali metal salt contained in the propellant powder to suppress muzzle flash.
- 2. The process of suppressing muzzle flash which comprises incorporating in propellant powder a small quantity of a potassium salt insufficient in itself to eliminate muzzle flash, and subsequently adding to the charge an increment of a potassium salt in quantity sufficient in combination with the potassium salt contained in the propellant powder to suppress muzzle flash.
- 3. The process of suppressing muzzle flash which comprises incorporating in propellant power a small quantity of potassium sulphate insufficient in itself to eliminate muzzle flash, and subsequently adding to the charge an increment of a potassium sulfate in quantity sufficient in combination with the potassium sulphate contained in the propellant powder to suppress the muzzle flash.
- 4. The process of suppressing muzzle flash which comprises incorporating in propellant power a small quantity of an alkali metal salt insufficient in itself to suppress muzzle flash, and subsequently adding to the propellant powder charge a cellulose ester colloid containing an alkali metal salt.
- 5. The process of claim 4 in which the alkali metal salt is a potassium salt.

6. The process of claim 4 in which the alkali metal salt is potassium sulphate.

7. A propellant powder charge comprising a propellant powder containing an alkali metal salt in insufficient quantity in itself to suppress muzzle flash in combination with a muzzle flash preventative increment containing sufficient alkali metal salt with that already present to suppress muzzle flash.

8. A propellant powder charge comprising a propellant powder containing potassium sulfate in insufficient quantity in itself to suppress muzzle flash in combination with a muzzle flash preventative increment containing potassium sulfate in sufficient quantity with that already present to suppress muzzle flash.

9. A propellant powder comprising nitrocellulose, a polynitrotoluene, a dialkylphthalate and an alkali metal salt in an amount less than 0.5 per cent in combination with a muzzle flash preventative increment containing an alkali metal salt in sufficient quantity with that already present to suppress muzzle flash.

10. A propellant powder comprising nitrocellulose, a polynitrotoluene, a dialkylphthalate and potassium sulfate in an amount less than 0.5 per cent in combination with a muzzle flash preventative increment containing potassium sulfate in sufficient quantity with that already present to suppress muzzle flash.

11. A propellant powder comprising nitrocellulose, dinitrotoluene, dibutylphthalate, a stabilizer, and an alkali metal salt in an amount less than 0.5 per cent in combination with a muzzle flash preventative increment containing potassium sulfate in sufficient quantity with that already present to suppress muzzle flash.

12. A propellant powder comprising nitrocellulose, dinitrotoluene, dibutylphthalate, and potassium sulfate in an amount less than 0.5 per cent in combination with a muzzle flash preventative increment containing potassium sulfate in sufficient quantity with that already present to suppress muzzle flash.

13. A muzzle flash preventative increment comprising a cellulose ester colloid containing incorporated therein a muzzle flash preventative alkali metal salt.

14. The product of claim 13 in which the alkali metal is potassium.

15. The product of claim 13 in which the alkali metal salt is potassium sulfate.

16. A muzzle flash preventative increment comprising a cellulose compound taken from a group consisting of a cellulose ether colloid, a cellulose ester colloid, and a cellulose nitrate colloid containing incorporated therein a muzzle flash preventative alkali metal salt.

17. The product of claim 16 in which the alkali metal is potassium.

18. The product of claim 16 in which the alkali metal salt is potassium sulfate.

19. A muzzle flash preventative increment comprising a cellulose nitrate colloid containing incorporated therein a muzzle flash preventative alkali metal salt.

5 20. The product of claim 19 in which the alkali metal is potassium.

21. The product of claim 19 in which the alkali metal salt is potassium sulfate.

16 22. A muzzle flash preventative increment comprising a cellulose nitrate colloid containing incorporated therein more than 10 per cent of a muzzle flash preventative alkali metal salt.

In testimony whereof, I affix my signature.

15 RICHARD GEORGE WOODBRIDGE.